

Jan. 3, 1939.

G. H. HOWE

2,142,846

METALLIC BOAT FOR USE IN HIGH TEMPERATURE FURNACES

Original Filed Sept. 17, 1937



Inventor:  
Goodwin H. Howe,  
by Harry E. Dunham  
His Attorney.

## UNITED STATES PATENT OFFICE

2,142,846

## METALLIC BOAT FOR USE IN HIGH TEMPERATURE FURNACES

Goodwin H. Howe, Scotia, N. Y., assignor to General Electric Company, a corporation of New York

Original application September 17, 1937, Serial No. 164,354. Divided and this application December 28, 1937, Serial No. 182,087

6 Claims. (Cl. 263—47)

The present invention is a division of my co-pending application Serial No. 164,354, filed September 17, 1937, and entitled Sintered alloy and method for making the same. In my prior application I have disclosed a furnace and method for fabricating from powdered materials alloys of the type disclosed in Ruder Patents 1,947,274 and 1,968,569, and Mishima Patents 2,027,994 to 2,028,000 inclusive. Alloys of this type, when made from powdered ingredients, are sintered in furnaces which employ a reducing atmosphere, such as hydrogen, and operate at temperatures in the neighborhood of 1400° C. The sintering chamber of such furnaces generally comprises an iron tube supported in an alundum tube which is electrically heated. In a continuous process for sintering alloys of the Ruder and Mishima type, it is desirable to employ metal boats on which the various pieces of material to be sintered may be positioned and then pushed through the furnace. Since the atmospheric conditions in the hot zone of the sintering section of the furnace is ideal for causing sticking of the boats to the iron tube, owing to the reducing action of the hydrogen and the high temperature employed, it is necessary to employ boats which avoid this difficulty.

It is an object of the present invention to provide a simple and economical form of metallic boat which will not stick to the iron tube portion of the furnace but which will permit free movement therethrough at the elevated temperatures.

The novel features which are characteristic of my invention are set forth with particularity in the appended claims. The invention itself however will best be understood from reference to the following specification when considered in connection with the accompanying drawing in which Fig. 1 is a longitudinal cross section of a boat employed in carrying out my invention, while Fig. 2 is a plan view of the boat illustrated in Fig. 1. In fabricating the boat which I have designated as a whole by the numeral 1, substantially pure iron powder is mixed with a smaller quantity of aluminum oxide powder, for example 75% iron and about 25% aluminum oxide and spread into a relatively thin even outer layer 2 having the surface dimensions required for the finished part. A second and thicker inner layer 3 of powdered iron is then superimposed on the first mentioned layer and the two layers pressed together in a mold and then sintered for about two hours at about 1450° C. Owing to the presence of the iron layer two or

more metal pieces thus fabricated may be readily welded together as indicated at 4 and 5 to thereby provide boats of any desired width and length. End pieces 6 and 7 having respectively oxide-iron mixtures 8 and 9 on the outside portions thereof are welded to the flat or base of the boat as indicated at 10 in Figs. 1 and 2.

A boat may be constructed entirely of the 25% aluminum oxide, 75% iron mixture but such material cannot be welded and unless a large enough mold is available to press a complete boat it is necessary to use pieces of composite construction having a weldable material on one side. A further advantage of using a composite boat is that any deformation of the boat due to alternate heating and cooling such as experienced in the process disclosed in applicant's prior application may be removed by cold pressing without danger of breakage or oxidation.

While I prefer to employ a mixture of about 75% iron and 25% aluminum oxide in the construction of the boat, these percentages are not critical and may be varied to a considerable extent. Furthermore, I may, if desired, employ in the construction of the boats a mixture of aluminum oxide or any other inert oxide with weldable metals other than iron. For example, if unusually high temperatures are to be employed in the sintering operation, metals such as tungsten, molybdenum and the like may be employed to replace the iron in part or if desired the iron may be replaced entirely by molybdenum.

What I claim as new and desire to secure by Letters Patent of the United States is:

1. A metal boat adapted to carry material through a furnace, said boat comprising a flat portion consisting of two superimposed layers, the outer layer consisting substantially of a mixture of weldable metal and an inert oxide and the inner layer consisting substantially of weldable metal.

2. A metal boat adapted to carry material through a furnace, said boat comprising a flat portion and an end portion, each of said portions consisting of two superimposed layers of material, the outer layer of said flat portion and the outer layer of said end portion consisting substantially of a mixture of a weldable metal and an inert oxide, and the inner layer of said flat portion and inner layer of said end portion consisting substantially of weldable metal.

3. A metal boat adapted to carry material through a furnace, said boat comprising two superimposed layers, the outer layer consisting of a mixture of iron and aluminum oxide and

the inner layer consisting substantially of iron.  
4. A metal boat adapted to carry material through a furnace, said boat comprising two superimposed layers, the outer layer consisting of 75% iron and 25% aluminum oxide, and the inner layer consisting of iron.

5. A metal boat adapted to carry material through a furnace, said boat comprising a flat portion and a vertical portion substantially at right angles thereto, each of said portions consisting of two superimposed layers, each outer layer consisting of a mixture of iron and alumi-

num oxide and each inner layer consisting substantially of iron.

6. A metal boat adapted to carry material through a furnace, said boat comprising a flat portion and a vertical portion substantially at right angles thereto, each of said portions consisting of two superimposed layers, each outer layer consisting of a mixture of about 75% iron and 25% aluminum oxide, and each inner layer consisting substantially of iron.

10

GOODWIN H. HOWE.